

## 1

2,993,336

OPERATION OF GAS TURBINE ENGINES AND  
FUEL COMPOSITIONS FOR USE IN SAID EN-  
GINES

Kenneth John Mackenzie, Eric Lewis Howe, and Richard Thomas Roles, all of Sunbury-on-Thames, England, assignors to The British Petroleum Company Limited, London, England, a joint-stock corporation of Great Britain

No Drawing. Filed Sept. 3, 1958, Ser. No. 758,668

Claims priority, application Great Britain Sept. 6, 1957

7 Claims. (Cl. 60—35.6)

This invention relates to a method for preventing or reducing the deterioration of a gas turbine engine, operating on a mineral oil residual fuel, particularly a petroleum residual fuel. This invention also relates to an improved fuel composition for use in gas turbine engines.

It is known that a gas turbine engine, operating on residual fuels containing mineral components, frequently deteriorates in condition and performance due to the accumulation of deposits within the engine, notably upon stator and rotor blades. In general, these deposits comprise sodium-containing compounds and vanadium-containing compounds. Furthermore it has been found that the lay-down of deposits is accompanied by corrosion of the underlying metal surfaces and thus removal of the deposits from the engine fails to restore completely the efficiency of said engine.

It has been stated that the class consisting of complex aluminium silicates provides suitable additives for residual fuel oils to provide fuel compositions for use in gas turbine engines; within this class of additive, felspar has been specifically proposed. We have found that within this broad class of additives consisting of complex aluminium silicates, specific compounds vary considerably in performance. In relation to a residual fuel which has not been treated with additive, the resulting fuel compositions will in some cases give an increased rate of build-up of deposits and in some cases may lead to a reduction in this build-up rate. However, providing that the rate of build-up of deposits does not exceed a limit which is set by economic factors, a major factor being required operating time between overhaul, this build-up rate is not regarded as the essential criterion of a good additive. It is considered that a factor of much greater importance is the rate of corrosion of the internal surfaces of the turbine, notably corrosion of rotor blades, since damage by corrosion cannot be remedied during routine overhaul and constitutes a serious limitation on effective engine life. We have found that within the broad class of complex aluminium silicates there is a sub-class of compounds which may be used as additives for residual fuels to provide improved fuel compositions. The improved compositions, when used in gas turbine engines, give a reduced rate of corrosion of internal surfaces of the turbine in comparison with the untreated fuel and also in comparison with compositions derived by the use of additives which, while being complex aluminium silicates, do not lie within the sub-class of compounds in accordance with the invention.

It is an object of this invention to provide an improved fuel composition for use in gas turbine engines. It is another object of this invention to provide an improved method of operating a gas turbine engine upon a residual fuel, of petroleum origin, containing vanadium. Other objects will appear hereinafter.

According to the present invention there is provided a fuel composition, suitable for use in gas turbine engines, containing a major proportion of a vanadium containing

## 2

residual fuel derived from petroleum and, in powder form, a minor proportion of a metal aluminium silicate complex having a mica crystalline structure. For brevity, said complex is hereinafter referred to as "mica."

5 Residual fuels employed in the compositions of this invention have a small content of vanadium which, under the conditions existing in a gas turbine engine and in the absence of additives, are converted to corrosive vanadium compounds. We have found that using a fuel composition containing "mica," the proportion of vanadium in combined form, in the deposits formed on the turbine blades is very small.

The preferred micas are muscovite (potassium mica) and phlogopite (magnesium mica); other micas which 15 may be employed are:

Paragonite (sodium mica)  
Lepidolite (lithium mica)  
Zinnwaldite (lithium-iron mica)  
Biotite (magnesium-iron mica)

20 Lepidomelane (iron micas containing ferric iron in large quantities)

The "mica" will normally be incorporated, in the fuel, in finely divided form whereby a suspension is formed.

25 Clearly the stability of the suspension will depend, among other factors, upon particle size, and preferably stirring means will be provided to maintain the composition.

According to a further aspect of the present invention 30 there is provided a method of operating a gas turbine engine upon a residual fuel, of petroleum origin, containing vanadium, by which damage or decline in efficiency due to corrosion is avoided or materially reduced wherein, during the operation of the engine on said fuel, a mica, in powder form, is introduced, continuously or intermittently, into the combustion chamber of said engine.

The optimum rate of feed of mica to the engine depend upon both the rate of feed of the fuel and upon the proportion of vanadium contained in the fuel. In general the use of mica in an amount constituting from 40 0.1% to 1.0% by weight of the fuel will be satisfactory; however the use of greater or smaller amounts also lies within the scope of this invention. When mica is added intermittently, greater amounts will usually be added during the period of injection but normally the amount so added, when averaged, over the injection cycle will not exceed 3% by weight of the fuel fed during this period.

The mica may be introduced into the engine by any desired method, including:

50 (a) Direct feed to the combustion zone by screw conveyor

(b) Introduction as a suspension in the fuel supply via the fuel injection nozzles

(c) Introduction as a suspension in bleed off stream 55 of the main fuel via subsidiary injection nozzles

(d) Introduction as a suspension in a liquid vehicle via subsidiary injection nozzles

(e) Introduction in "fluidised" state into (i) the total air stream to the combustion chamber, or (ii) the air 60 stream to the primary zone that is, the zone containing the main fuel jet or jets, in which combustion is initiated or (iii) the air stream to the dilution zone, that is the zone to which air is admitted for the purpose of reducing the temperature of the combustion products.

A modified gas turbine engine having subsidiary injection nozzles, suitable for introducing a mica in suspension according to the present invention, is described in British Patent Specification No. 779,248.

Of the methods hereinbefore described, methods (b) 70 and (e) are preferred.

As hereinbefore stated, the additive may be introduced into the engine in intermittent manner. Preferably the mica will be introduced over a period of hours by one or other of the methods described and thereafter a substantial measure of protection from corrosion will be achieved notwithstanding that residual fuel free of corrosion preventing additive is employed. After a period of hours of operation under these conditions the cycle will be repeated.

Preferably in a cycle of operations the mica is introduced for a period not exceeding 20 hours and thereafter the engine is operated without introduction of mica for a period of at least 80 hours. By way of illustration the cycle may consist of 12 hours' operation with injection of mica at the rate of 0.1-1.0% by weight of the residual fuel followed by 88 hours' operation using residual fuel without mica injection to the engine.

By intermittent injection of mica, as described, the rate of build-up of deposits (during the operational cycle) will be less than is the case when the same amount of mica is continuously injected; nevertheless good resistance to corrosion will be achieved.

This invention is illustrated but in no way limited by the following example.

An experimental gas turbine combustion rig was employed to test a series of fuel compositions. The combustion rig was of the following construction:

- (a) A compressor providing up to 2 pounds of air per second at 3-4 p.s.i.g.
- (b) A pre-heating combustion chamber to raise the air temperature to 350° C.
- (c) The main residual oil burning combustion chamber.
- (d) A test blade section consisting of four turbine stator blades arranged to simulate the first row of turbine blading.
- (e) Instrumentation, fuel systems and general auxiliaries.

To simulate the air temperature conditions of an industrial gas turbine engine, in which compressed air

gas stream and the weight of deposit found by difference. To measure corrosion, the test blades were descaled in the following manner:

The blades were immersed in a boiling mixture of 30 percent weight caustic soda, 2 percent weight potassium permanganate and 68 percent water for one hour after which they were scrubbed under running water with a brass wire brush. The blades were then replaced in the mixture for a second hour and the scrubbing treatment repeated. Water vaporisation losses from the mixture were made good by topping up with distilled water. After the second scrubbing treatment the blades were replaced for two minutes in a mixture of 1 part concentrated nitric acid and 3 parts water to which had been added 1 percent volume of 90/100 volume hydrogen peroxide. The temperature of this mixture was maintained at 60° C. On removal the blades were washed under running water, then in acetone and dried ready for weighing.

20

#### EXAMPLE 1

Tests 1 and 2 are provided by way of comparison. In test 1, the fuel employed was a kerosine distillate fraction of petroleum origin. In test 2 and test 3 the fuel employed was an Admiralty Reference Fuel, having the code name "Mothball," of the following characteristics:

Viscosity (Redwood No. 1 at 100° F.) secs 635  
 30 Ash percent 0.058  
 Vanadium content p.p.m. 258  
 Sodium content p.p.m. 1

In test 3 mica was injected into the total air supply to the combustion chamber. The mica used was muscovite (potassium aluminium silicate complex) and had a particle size such that 80% passed through a 200 British Standard mesh.

Test conditions and results obtained are shown in the following Table 1.

TABLE 1

| Test No. | Fuel     | Test Duration, Hr. | Average gas temperature at entry to test blades, ° C. | Additive Injection Material and Flow | Blade Weight Increase during test (fouling), mg. | Blade Weight Metal loss (corrosion), mg. |
|----------|----------|--------------------|-------------------------------------------------------|--------------------------------------|--------------------------------------------------|------------------------------------------|
| 1        | Kerosine | 12                 | 650                                                   | Nil                                  | 1.4                                              | 51.0                                     |
| 2        | Mothball | 12                 | 650                                                   | Nil                                  | 51.0                                             | 144.0                                    |
| 3        | do       | 12                 | 650                                                   | Mica 0.3% on fuel flow.              | 220.0                                            | 72.0                                     |

would be preheated by a heat exchanger, there was provided a preheating chamber through which the flow of compressed air passed before reaching the main combustion chamber; the preheating chamber was in the form of a refractory lined combustion chamber and was equipped with a medium air pressure atomizing nozzle, operating on kerosine.

A jig, hereinafter referred to as the test blade holder, and constructed to locate four turbine blades in the relative positions in which they would be mounted in a rotor, was carried on the rig in such manner that it slid from a position clear of the exhaust gas stream into a second position in which, by means of ducting, this gas stream was directed over the test blades. Under the conditions of test employed, the two outer blades served as guide vanes for ensuring normal flow (as would occur during operation of a turbine) over the two inner blades. The blade holder was brought into position for test purposes after steady operating conditions had been established. To measure fouling, the inner blades were weighed both before and after exposure to the exhaust

55

Operational runs were carried out in pairs in the apparatus described in Example 1. In the first run a reference fuel was employed without additive; in the second run a fuel composition was employed which contained reference fuel together with the additive. Measurements were made of the increase in weight (fouling) of the test blades and of the weight of the blades after cleaning. Results are expressed as (a) percentage difference (increase or decrease) in fouling, in relation to fouling obtained using fuel without additive and (b) percentage reduction in corrosion (loss of weight of the blades after cleaning) in relation to corrosion obtained using fuel without additive.

The reference fuel was the fuel known as Admiralty Reference Fuel "Vanilla" which has an ash content of 0.08% by weight, a vanadium content of 360 parts per million and a viscosity (Redwood No. 1 at 100° F.) of 650 seconds.

In all the runs the test blade temperature was held at 750° C.

Other conditions and results obtained are shown in the following Table 2.

of said engine and constitutes 0.1-3% by weight of the residual fuel.

TABLE 2

| Test No. | Test Duration, Hr. | Additive                             | Injection Position and Rate                                              | Percentage Difference in fouling (by weight) | Percentage Reduction in corrosion (by weight) |
|----------|--------------------|--------------------------------------|--------------------------------------------------------------------------|----------------------------------------------|-----------------------------------------------|
| 321..... | 12                 | Muscovite Mica (Slurry in Lub. Oil). | Into High Pressure Fuel Pump Suction. .33% by weight Mica on Fuel Flow.  | 4.0 Increase.....                            | 23.0                                          |
| 313..... | 12                 | Powdered Muscovite Mica.             | Primary Zone. .33% by weight on Fuel Flow.                               | 32.0 Increase.....                           | 32.0                                          |
| 294..... | 12                 | do.....                              | Primary Zone. 1.70% by weight on Fuel Flow.                              | 575.0 Increase.....                          | 50.0                                          |
| 303..... | 100                | do.....                              | Primary Zone. 1.7% by weight on fuel flow for first 12 hr. of test only. | 26.0 Increase.....                           | 53.0                                          |
| 319..... | 12                 | Powdered Phlogopite Mica.            | Primary Zone. .33% by weight on fuel flow.                               | 22.0 Reduction.....                          | 16.5                                          |
| 314..... | 12                 | Powdered Felspar.                    | do.....                                                                  | 72.0 Reduction.....                          | Nil                                           |

We claim:

1. A fuel composition, suitable for use in gas turbine engines, containing a major proportion of a vanadium containing residual fuel derived from petroleum and, in powder form, 0.1-3% by weight of the residual fuel of a metal aluminium silicate complex having a mica crystalline structure.

2. A fuel composition as specified in claim 1 in which the mica is muscovite.

3. A fuel composition as specified in claim 1 in which the mica is phlogopite.

4. A fuel composition as specified in claim 1 in which the metal aluminium silicate complex constitutes 0.1 to 1.0% by weight of the residual fuel.

5. A method of operating a gas turbine engine upon a residual fuel, of petroleum origin, containing vanadium, wherein damage or decline in efficiency due to corrosion is avoided or materially reduced wherein, during the operation of the engine on said fuel, metal aluminium silicate complex, having a mica crystalline structure, is introduced, in powder form, into the combustion chamber

6. A method as specified in claim 5 in which the metal aluminium silicate complex constitutes 0.1 to 1.0% by weight of the residual fuel.

7. A method as specified in claim 5 in which the metal aluminium silicate complex is introduced intermittently and in which in a cycle of operation said complex is introduced for a period not exceeding 20 hours and thereafter the engine is operated without introduction of said complex for a period of at least 80 hours.

#### References Cited in the file of this patent

#### FOREIGN PATENTS

|         |               |                |
|---------|---------------|----------------|
| 314,443 | Switzerland   | July 31, 1956  |
| 315,324 | Switzerland   | Sept. 29, 1956 |
| 200,149 | Australia     | Nov. 4, 1955   |
| 201,884 | Australia     | May 24, 1956   |
| 740,062 | Great Britain | Nov. 9, 1955   |
| 745,012 | Great Britain | Feb. 15, 1956  |
| 762,521 | Great Britain | Nov. 28, 1956  |